

Patented Dec. 6, 1927.

## UNITED STATES PATENT OFFICE.

GEORG WELTER, OF FRANKFORT-ON-THE-MAIN, GERMANY, ASSIGNOR, BY MESNE ASSIGNMENTS, TO ALLIED PROCESS CORPORATION, OF NEW YORK, N. Y., A CORPORATION OF NEW YORK.

## LITHIUM-CONTAINING BEARING METALS.

No Drawing. Application filed March 6, 1925, Serial No. 13,633, and in Germany March 12, 1924.

It has been found that alloys consisting essentially of lead alloyed with relatively small amounts of lithium and sodium, or lithium and potassium, or lithium, sodium and potassium, possess, as compared with known bearing-metals, particularly valuable properties. Such alloys containing only a very small amount of lithium exhibit a comparatively great hardness or 10 rigidity and possess in addition to a high resistivity to shocks, good casting qualities, and low melting point, a characteristically high compression strength, being in this respect approximately equivalent to red brass. 15 Such alloys also possess excellent bearing properties.

Lead alloys containing potassium and lithium each in quantity amounting to less than 1%, have particularly favorable bearing 20 qualities fitting them for use in heavy duty bearings.

Lead alloys containing sodium and lithium, each in quantity amounting to less than 1%, are characterized by their great resist- 25 tivity against shocks, in view of which their use in bearings subject to shocks is indicated.

By alloying lead with lithium and both sodium and potassium, each in quantity not exceeding 1%, a combination of the qualities referred to may be obtained. The proportions of the additions, lithium, sodium and potassium, may be varied to produce alloys having the desired qualities or combination of qualities. For example, alloys containing up to about 0.8% of sodium and up to about 0.8% of potassium and up to 30 about 0.1% of lithium and the remainder consisting principally of lead, are very useful as bearing-metals for general applica- 35 tion.

All of the alloys above referred to may contain, besides the lead and the sodium, potassium and lithium additions, small 40 quantities of other elements such as copper, nickel, cobalt, zinc, magnesium, strontium, calcium mercury phosphorus and sulfur. The effects of these elements in bearing-metal alloys consisting essentially of 45 lead are generally known and their use to secure particular properties is within the skill of the technologist. The quantities of such additions generally should not exceed 50 about 5% in the aggregate.

The alloys of the present invention are less susceptible to corrosion than the known bearing-metal alloys containing alkaline earth metal additions. By suitable surface treatment, for instance by tinning, the resistivity of the alloys against corrosion may be further improved.

The alloys can be produced according to any of the known methods, for instance by melting the components or alloys thereof together, electrolysis, diffusion, etc.

As is apparent from the foregoing, the invention resides principally in the addition of lithium to bearing-metal alloys consisting essentially of lead and containing other alkali metals, with or without other known 70 additions or components such as the alkaline earth and the heavy metals. The lithium besides conferring valuable physical properties, reduces the total alkali metal content of the alloy required, and as a result reduces 75 the tendency of the alloys to corrode.

## I claim:

1. Bearing-metal alloys consisting essentially of lead and comprising lithium in quantity sufficient to produce an appreciable 80 hardening effect but not in excess of about 0.1% and an appreciable amount of at least one other alkali metal not substantially in excess of about 1.0%.

2. Bearing-metal alloys consisting essen- 85 tially of lead and comprising lithium in quantity sufficient to produce an appreciable hardening effect but not in excess of about 0.1% and an appreciable amount of sodium not substantially in excess of about 1.0%. 90

3. Bearing-metal alloys consisting essen- 95 tially of lead and comprising lithium in quantity sufficient to produce an appreciable hardening effect but not in excess of about 0.1% and an appreciable amount of sodium not substantially in excess of about 1.0%, and an appreciable amount of potassium not substantially in excess of about 1.0%. 100

4. Bearing-metal alloys consisting essen- 100 tially of lead and comprising lithium in quantity sufficient to produce an appreciable hardening effect but not in excess of about 0.1%, an appreciable amount of at least one other alkali metal not substantially in excess of about 1.0% and an appreciable amount of an alkaline earth metal not substantially in excess of about 1.0%. 105

5. Bearing-metal alloys consisting essen-

tially of lead and comprising lithium in quantity sufficient to produce an appreciable hardening effect but not in excess of about 0.1%, an appreciable amount of sodium not substantially in excess of about 1.0% and an appreciable amount of an alkaline earth metal not substantially in excess of about 1.0%.

6. Bearing-metal alloys consisting essentially of lead and comprising lithium in quantity sufficient to produce an appreciable hardening effect but not in excess of about 0.1%, an appreciable amount of sodium not substantially in excess of about 1.0%, an appreciable amount of potassium not substantially in excess of about 1.0%, and an appreciable amount of an alkaline earth metal not substantially in excess of about 1.0%.

7. Bearing-metal alloys consisting essentially of lead and comprising lithium in quantity sufficient to produce an appreciable

hardening effect but not in excess of about 0.1%, an appreciable amount of sodium not substantially in excess of about 1.0%, an appreciable amount of potassium not substantially in excess of about 1.0%, and an appreciable amount of calcium not substantially in excess of about 1.0%.

8. Bearing-metal alloys consisting of about 95% of lead, lithium in quantity sufficient to produce an appreciable hardening effect but not in excess of about 0.1%, an appreciable amount of at least one other alkali metal not substantially in excess of about 1.0%, an alkaline earth metal in an appreciable amount not substantially in excess of about 1.0%, and at least one of the elements copper, nickel, cobalt, zinc, magnesium, phosphorus and sulfur.

In testimony whereof, I affix my signature.

GEORG WELTER.